# EUROPEAN PATENT SPECIFICATION

(11) **EP 2 230 670 B1**
(45) Date of publication and mention of the grant of the patent: **16.11.2011**
(21) Application number: 09155274.5
(22) Date of filing: 16.03.2009
(51) Int. Cl.: H01B 3/44

(54) **Medium voltage cable**
Mittelspannungskabel
Câble de moyenne tension

(43) Date of publication of application: 22.09.2010
(73) Proprietor: Trelleborg Forsheda Building AB, 331 29 Värnamo (SE)
(72) Inventor: Svensson, Panch, 331 33, Värnamo (SE)
(74) Representative: Hjalmarsson, Magnus Axel

(56) References cited:
- EP-A- 1 176 161
- CA-C- 2 220 495
- US-A1- 2006 052 511

## Description

### Field of the invention

The present invention relates to a medium-voltage cable comprising a conductive cable core, an insulation layer for insulating the cable core, and an outer semiconductive insulation shield.

### Background of the invention

A cable for transmitting medium-voltage, i.e. 5-49 kV, electrical power comprises at least one conductive cable core, which is covered by a polymer layer for insulation. The polymer layer normally comprises at least three layers:
a) an inner, relatively thin semiconductive layer;
b) a relatively thick insulating layer, outside the inner semiconductive layer; and
c) an outer, relative thin semiconductive layer, forming an insulation shield, outside the insulating layer.

The purpose of the semiconductive layers is to distribute the electrical field across the insulating layer over the cable surface, which reduces the risk of disruptive breakdown damaging the insulating layer. For such purposes, the semiconductive layers should have a volume resistivity, as measured according to the standard ASTM D257, of from 10 Ohm.cm to 20 000 Ohm.cm, which is used as the definition of "semiconductive" throughout this disclosure. Any granulate or compound for forming such a layer may, of course, have a resistivity outside this range, and still be viable for forming a semiconductive layer having a resistivity within this range.

The polymer layer, i.e. the insulating and semiconductive layers, should preferably be stable over time, and resistant to heat and humidity. For some applications, and in some markets, there is also a need for cables allowing the outer semiconductive layer to be stripped from the insulator. Such cables normally have an insulator of either an ethylene-propylene rubber (EPR) copolymer, or of a crosslinked polyethylene homopolymer (commonly abbreviated PEX or XLPE), as several polymers suitable for semiconductive layers, exhibiting strippability from those insulators, are known and readily available.

There are some drawbacks with known cables having a strippable semiconductive layer. For example, EPR is expensive; it generally costs about twice as much as polyethylene, and the extrusion of EPR consumes more energy than extrusion of PEX. Insulating layers of PEX homopolymers, on the other hand, are susceptible to water-tree formation as they are exposed to humidity and high voltages over time, thereby reducing the life expectancy of the cable and increasing the risk of a disruptive breakdown. This is to some extent compensated for by adding water-tree retardants (WTR) to the insulator. Unfortunately, extrusion of WTR-PEX can be troublesome, as many WTR additives are prone to leave deposits in processing equipment, thereby increasing the needed frequency of production stoppages for cleaning the equipment.

The predominant material for strippable semiconductive layers on EPR and water-tree resistant PEX insulators is a copolymer of ethylene vinyl acetate (EVA), mixed with nitrile-butadiene rubber (NBR) and carbon black. "Strippable shields with Improved Thermal Stability and Faster Cable Extrusion Rate", 6^{th} International Conference on Insulated Power Cables, JICABLE '03, describes the current state-of-the-art regarding semiconductive compounds that are strippable from a water-tree resistant crosslinked polyethylene insulator.
EP 1176161 discloses a conductive wire coated with a composition of a crosslinked blend of polyethylene with an ethylene - alkyl acrylate copolymer.
US 2006/052511 discloses compositions comprising ethylene - ethyl acrylate - carbon monoxide terpolymers.

### Summary of the invention

It is an object of the present invention to solve, or at least mitigate, parts or all of the above mentioned problems. To this end, there is provided a cable for transmitting electrical power at a voltage between 5 and 49 kV, the cable comprising
a conductive cable core;
an insulation layer for insulating the cable core, the insulation layer comprising from 50 to 90% of crosslinked polyethylene, and from 10 to 50% of at least one copolymer selected from the group consisting of ethylene-alkyl acrylates and ethylene vinyl acetate; and
an outer semiconductive screen, forming an outer layer on the insulation layer, and comprising from 30 to 70% by weight of a composition (A) of at least one copolymer selected from the group consisting of ethylene-alkyl acrylate carbon monoxides. Thanks to the invention, a strippable semiconductive screen may be provided on a relatively inexpensive water-tree resistant cable insulator, without the drawbacks of WTR additives.

Preferably, the outer semiconductive screen presents an adhesion to the insulation layer of from 5 to 50 N/cm, and more preferably from 10 to 30 N/cm.

In one embodiment, the cable comprises an inner semiconductive layer between the conductive cable core and the insulation layer, the inner semiconductive layer comprising from 30 to 70% by weight of said composition (A). By using essentially the same material for the inner semiconductive layer, inventory management, mixing of compositions, and extrusion can be simplified.

Preferably, said at least one copolymer selected from the group consisting of ethylene-alkyl acrylate carbon monoxides, of said composition (A), comprises from 25 to 70% by weight of ethylene; from 25 to 50% by weight of at least one alkyl acrylate; and from 5 to 25% by weight of carbon monoxide. Those intervals have been found to yield a suitable level of adhesion.

Preferably, an alkyl of said at least one copolymer selected from the group consisting of ethylene-alkyl acrylate carbon monoxides, of said composition (A), is butyl, since ethylene butyl acrylate carbon monoxide has a high polarity, thereby resulting in a high strippability, while being readily available on the market.

Preferably, the polyethylene of the insulator is a low-density polyethylene (LDPE), as those have proven particularly suitable for medium voltage cable insulators.

In one preferred embodiment, the outer semiconductive screen further comprises from 5 to 30% by weight of NBR; and from 30 to 40% by weight of carbon black. The use of a substantial fraction of NBR in the semiconductive screen improves its viscosity, and thereby makes it easier to extrude. Furthermore, by adding a carefully selected amount of NBR, also the adhesion of the semiconductive layer to the insulator can be adjusted.

According to another aspect of the invention, parts or all of the above mentioned problems are solved, or at least mitigated, by a polymer mixture for preparing an outer semiconductive screen for a cable, the mixture comprising from 5 to 30% by weight of NBR; from 30 to 40% by weight of carbon black; and from 30 to 70% by weight of a composition (A) of at least one copolymer selected from the group consisting of ethylene-alkyl acrylate carbon monoxides. Thanks to the invention, a strippable semiconductive screen having good extrusion properties may be provided on a relatively inexpensive water-tree resistant cable insulator.

Preferably, said at least one copolymer selected from the group consisting of ethylene-alkyl acrylate carbon monoxides, of said composition (A), comprises from 25 to 70% by weight of ethylene; from 25 to 50% by weight of at least one alkyl acrylate; and from 5 to 25% by weight of carbon oxide.

Preferably, an alkyl of said at least one copolymer selected from the group consisting of ethylene-alkyl acrylate carbon monoxides, of said composition (A), is butyl.

### Brief description of the drawing

The above, as well as additional objects, features and advantages of the present invention, will be better understood through the following illustrative and non-limiting detailed description of a preferred embodiment of the present invention, with reference to the appended drawing, wherein:
Fig. 1 is a diagrammatic view in section of a medium-voltage cable.

### Detailed description of the exemplary embodiments

The introduction briefly describes current state-of-the-art in the field of water-tree resistant insulators for strippable semiconductive coatings. In the field of cables with non-strippable semiconductive layers, on the other hand, water-tree formation is generally not a problem, since the composition of the insulation layer can be made without regard to the strippability of an outer semiconductive layer. Insulators of non-strippable cables usually comprise a terpolymer of either EVA (ethylene-vinyl acetate) or EEA (ethylene-ethyl acrylate), and ethylene. Such a terpolymer is not prone to forming water-trees, but on the other hand results in a permanently bonded semiconductive shield. Detailed descriptions on how such insulating layers may be composed are given in EP 1916672 A1.

Fig. 1 illustrates a medium-voltage cable, i.e. a cable for electrical power transmission applications in the range 5-49 kV. The cable 10 comprises a central conductor 12 made of stranded copper wires 12'. A first, inner semiconductive layer 14 is deposited directly onto the conductor 12. The inner semiconductive layer 14 serves for smoothing the conductor's 12 interface towards an insulator layer 16, which electrically insulates the conductor 12 and the inner semiconductive layer 14 from the electrical (ground) potential surrounding the cable 10. A second, outer semiconductive layer 18 is deposited onto the insulator layer 16. The outer semiconductive layer 18 serves for distributing the electrical field, which is present across the insulator 16 when a voltage is applied to the conductor 12, evenly over the insulator area. Additional layers 20, such as water barriers and/or jackets for mechanical protection, may be present outside the outer semiconductive layer 18.

The outer semiconductive layer 18 is strippable from the insulator layer 16, such that the outer semiconductive layer 18 may be removed from the insulator layer 16 without significantly damaging the surface of the insulator layer 16, and without leaving any significant residues of semiconductive polymer on the surface of the insulator layer 16 after stripping. Strippable is, in this disclosure, defined as having an adhesion of from 5 to 50 N/cm, measured as the force required to peel off a strip of the outer semiconductive layer 18, cut to a width of 1 cm, from the surface of the insulator 16, while pulling at a speed of 50 mm/min. This method of measuring is described in more detail in the AFNOR standard NF C33-223. Ideally, the adhesion should however be in the range 10 to 30 N/cm for optimal strippability.

The insulating layer 16 consists of an LDPE-EEA copolymer that is formed by cross-linking a compound that consists of about 80% by weight of low-density polyethylene (LDPE), wherein low-density is defined as being in the range 0.910 - 0.940 g/cm³, and 20% by weight of ethylene-ethyl acrylate (EEA). A peroxide is used as a cross-linking agent. The EEA component effectively counteracts the formation of water-trees. An example of a suitable ethylene-ethyl acrylate compound consists of 10% ethylene, and 90% ethyl acrylate. An example of a suitable LDPE is Borealis SuperCure LC8205R, which is in fact intended for use with permanently bonded insulation shields. However, even though less preferred, also other types of polyethylenes, e.g. high-density polyethylene (HDPE), can be used instead of LDPE. The polyethylene may be cross-linked with other components instead of or in combination with EEA, e.g. ethylene butyl acrylate (EBA) and/or other ethylene-alkyl acrylates (EAA), and/or ethylene vinyl acetate (EVA) for applications having less demanding requirements on heat stability during vulcanization.

The inner and outer semiconductive layers 14, 18 consist of a mixture of 30% by weight of carbon black, 20% by weight of nitrile-butadiene rubber (NBR), and 50% by weight of a terpolymer of ethylene, butyl acrylate, and carbon monoxide (EBA-CO).

A suitable carbon black for the semiconductive composition above is Cabot Corporation's Vulcan XC500.

Preferably, the NBR is an acrylonitrile-butadiene rubber having a high content, ideally 35-50%, of acrylonitrile (ACN). An example of an NBR that is suitable for the semiconductive composition above, and having an ACN content of 44%, is Perbunan 4456F, available from LAXNESS Deutschland GmbH. The NBR serves for adjusting the viscosity of the rubber mix, thereby making it easier to extrude, but also contributes to the strippability of the mix. However, it is the EBA-CO that is the key ingredient for strippability, making it possible to obtain a semiconductive coating that is strippable from an insulator that consists of a copolymer of EVA and/or EAA, and PEX.

A suitable EBA-CO is an ethylene n-butyl acrylate carbon monoxide (EnBA-CO), sold by Dupont under the trade name Elvaloy HP661.

A semiconductive layer formed from the compound of EnBA-CO, carbon black and NBR described in detail above, co-extruded onto an insulator of LDPE-EEA according to the description hereinbefore, presents an adhesion of about 18 N/cm. By varying the process parameters of the extrusion and vulcanization, it is possible to vary this adhesion somewhat; greater variations may of course be obtained by varying the relative proportions of the constituents in the composition. EBA-CO, compared to e.g. EVA, also offers a higher resistance to heat during vulcanization, thereby allowing for faster extrusion, leading to a higher production speed and a lower cost per produced meter of cable.

Instead of, or in combination with EBA-CO, but somewhat less preferred due to higher cost or less abundant availability on the market, also other ethylene-alkyl acrylate carbon monoxide (EAA-CO) copolymers can be used for achieving a strippable semiconductive layer. Preferably, the EAA-CO comprises at least one copolymer selected from the group consisting of ethylene-alkyl acrylate carbon monoxides. Preferably, said at least one copolymer selected from the group consisting of ethylene-alkyl acrylate carbon monoxides comprises from 25 to 70% by weight of ethylene; from 25 to 50% by weight of at least one alkyl acrylate; and from 5 to 25% by weight of carbon oxide. Alkyls that are particularly preferred for use in an EAA-CO compound that is to be used for semiconductive layers that are strippable from copolymer isolators of the mentioned types are, e.g., methyl, ethyl, propyl, butyl, pentyl and hexyl, of which methyl, ethyl and butyl are more preferred, and butyl is the most preferred as it is relatively highly polar and readily available at a reasonable cost.

The invention has mainly been described above with reference to a few embodiments. However, as is readily appreciated by a person skilled in the art, other embodiments than the ones disclosed above are equally possible within the scope of the invention, as defined by the appended patent claims.

For example, NBR, even though it contributes to the strippability to some extent, is not an essential component in a strippable semiconductive coating. It is preferred, though, since it improves the extrusion properties, such as the viscosity, of the composition.

Also other types of carbon black than Vulcan XC500 may, obviously, be used for obtaining the correct resistivity of the semiconductive layer, but the fraction of carbon black in the semiconductive material may need to be adjusted accordingly.

The semiconductive polymer mixture described in detail hereinbefore may also be applied to other insulator compositions than those described in detail above; strippability is also obtained when applied to insulators of EPR and/or polyethylene homopolymers.

## Claims

1. A cable for transmitting electrical power at a voltage between 5 and 49 kV, comprising
a conductive cable core (12);
the cable being **characterized in**
an insulation layer (16) for insulating the cable core (12), the insulation layer (16) comprising
from 50 to 90% of polyethylene, and
from 10 to 50% of at least one copolymer selected from the group consisting of ethylene-alkyl acrylates and ethylene vinyl acetate; and
an outer semiconductive screen (18), forming an outer layer on the insulation layer (16), and comprising from 30 to 70% by weight of a composition (A) of at least one copolymer selected from the group consisting of ethylene-alkyl acrylate carbon monoxides.

2. A cable according to claim 1, wherein the outer semiconductive screen (18) presents an adhesion to the insulation layer (16) of from 5 to 50 N/cm, and more preferably from 10 to 30 N/cm.

3. A cable according to any of the previous claims, further comprising an inner semiconductive layer (14) between the conductive cable core (12) and the insulation layer (16), the inner semiconductive layer (14) comprising from 30 to 70% by weight of said composition (A).

4. A cable according to any of the previous claims, wherein said at least one copolymer selected from the group consisting of ethylene-alkyl acrylate carbon monoxides, of said composition (A), comprises
from 25 to 70% by weight of ethylene;
from 25 to 50% by weight of at least one alkyl acrylate; and
from 5 to 25% by weight of carbon monoxide.

5. A cable according to any of the previous claims, wherein an alkyl of said at least one copolymer selected from the group consisting of ethylene-alkyl acrylate carbon monoxides, of said composition (A), is butyl.

6. A cable according to any of the previous claims, wherein said polyethylene is a low-density polyethylene.

7. A cable according to any of the previous claims, wherein the outer semiconductive screen (18) further comprises
from 5 to 30% by weight of NBR; and
from 30 to 40% by weight of carbon black.

8. A polymer mixture for preparing an outer semiconductive screen for a cable, comprising
from 5 to 30% by weight of NBR;
from 30 to 40% by weight of carbon black; and
from 30 to 70% by weight of a composition (A) of at least one copolymer selected from the group consisting of ethylene-alkyl acrylate carbon monoxides.

9. A polymer mixture according to claim 8, wherein said at least one copolymer selected from the group consisting of ethylene-alkyl acrylate carbon monoxides, of said composition (A), comprises
from 25 to 70% by weight of ethylene;
from 25 to 50% by weight of at least one alkyl acrylate; and
from 5 to 25% by weight of carbon oxide.

10. A polymer mixture according to any of the claims 8-9, wherein an alkyl of said at least one copolymer selected from the group consisting of ethylene-alkyl acrylate carbon monoxides, of said composition (A), is butyl.

## Patentansprüche

1. Kabel zum Übertragen von elektrischem Strom bei einer Spannung zwischen 5 und 49 kV, das Folgendes umfasst:
einen leitfähigen Kabelkern (12);
wobei das Kabel **gekennzeichnet ist durch**
eine Isolierungsschicht (16) zum Isolieren des Kabelkerns (12), wobei die Isolierungsschicht (16) Folgendes umfasst:
50 bis 90 % Polyethylen, und
10 bis 50 % mindestens eines Copolymers, das aus der Gruppe bestehend aus Ethylenalkylacrylaten und Ethylenvinylacetat ausgewählt ist; und
eine äußere halb-leitfähige Abschirmung (18), die eine äußere Schicht auf der Isolierungsschicht (16) bildet und 30 bis 70 Gewichts-% einer Zusammensetzung (A) aus mindestens einem Copolymer, das aus der Gruppe bestehend aus Ethylenalkylacrylat-Kohlenmonoxiden ausgewählt ist, umfasst.

2. Kabel nach Anspruch 1, wobei die äußere halb-leitfähige Abschirmung (18) eine Adhäsion für die Isolierungsschicht (16) von 5 bis 50 N/cm und besonders bevorzugt 10 bis 30 N/cm bereitstellt.

3. Kabel nach einem der vorangehenden Ansprüche, das des Weiteren eine innere halb-leitfähige Schicht (14) zwischen dem leitfähigen Kabelkern (12) und der Isolierungsschicht (16) umfasst, wobei die innere halb-leitfähige Schicht (14) 30 bis 70 Gewichts-% der Zusammensetzung (A) umfasst.

4. Kabel nach einem der vorangehenden Ansprüche, wobei das mindestens eine, aus der Gruppe bestehend aus Ethylenalkylacrylat-Kohlenmonoxiden ausgewählte Copolymer der Zusammensetzung (A) Folgendes umfasst:
25 bis 70 Gewichts-% Ethylen;
25 bis 50 Gewichts-% mindestens eines Alkylacrylats; und
5 bis 25 Gewichts-% Kohlenmonoxid.

5. Kabel nach einem der vorangehenden Ansprüche, wobei ein Alkyl des mindestens einen, aus der Gruppe bestehend aus Ethylenalkylacrylat-Kohlenmonoxiden ausgewählten Copolymers der Zusammensetzung (A) Butyl ist.

6. Kabel nach einem der vorangehenden Ansprüche, wobei das Polyethylen ein Polyethylen von geringer Dichte ist.

7. Kabel nach einem der vorangehenden Ansprüche, wobei die äußere halb-leitfähige Abschirmung (18) des Weiteren Folgendes umfasst:
5 bis 30 Gewichts-% NBR; und
30 bis 40 Gewichts-% Ruß.

8. Polymergemisch zur Herstellung einer äußeren halb-leitfähigen Abschirmung für ein Kabel, das Folgendes umfasst:
5 bis 30 Gewichts-% NBR;
30 bis 40 Gewichts-% Ruß; und
30 bis 70 Gewichts-% einer Zusammensetzung (A) aus mindestens einem Copolymer, das aus der Gruppe bestehend aus Ethylenalkylacrylat-Kohlenmonoxiden ausgewählt ist.

9. Polymergemisch nach Anspruch 8, wobei das mindestens eine, aus der Gruppe bestehend aus Ethylenalkylacrylat-Kohlenmonoxiden ausgewählte Copolymer der Zusammensetzung (A) Folgendes umfasst:
25 bis 70 Gewichts-% Ethylen;
25 bis 50 Gewichts-% mindestens eines Alkylacrylats; und
5 bis 25 Gewichts-% Kohlenoxid.

10. Polymergemisch nach einem der Ansprüche 8-9, wobei ein Alkyl des mindestens einen, aus der Gruppe bestehend aus Ethylenalkylacrylat-Kohlenmonoxiden ausgewählten Copolymers der Zusammensetzung (A) Butyl ist.

## Revendications

1. Câble pour transmettre de l'énergie électrique à une tension entre 5 et 49 kV, comprenant :
une mèche de câble conductrice (12) ;
le câble étant **caractérisé par**:
une couche isolante (16) pour isoler la mèche de câble (12), la couche isolante (16) comprenant:
de 50 à 90 % de polyéthylène, et
de 10 à 50 % d'au moins un copolymère sélectionné dans le groupe se composant d'acrylates d'éthylène-alkyle et d'acétate d'éthylène de vinyle; et
un écran semi-conducteur extérieur (18) constituant une couche extérieure sur la couche isolante (16) et comprenant de 30 à 70 % en poids d'une composition (A) d'au moins un copolymère sélectionné dans le groupe se composant de monoxydes de carbone d'acrylates d'éthylène-alkyle.

2. Câble selon la revendication 1, dans lequel l'écran semi-conducteur extérieur (18) présente une adhérence à la couche isolante (16) de 5 à 50 N/cm, et de préférence de 10 à 30 N/cm.

3. Câble selon l'une quelconque des revendications précédentes, comprenant en outre une couche semi-conductrice intérieure (14) entre la mèche de câble conductrice (12) et la couche isolante (16), la couche semi-conductrice intérieure (14) comprenant de 30 à 70 % en poids de ladite composition (A).

4. Câble selon l'une quelconque des revendications précédentes, dans lequel ledit au moins un copolymère sélectionné dans le groupe se composant de monoxydes de carbone d'acrylates d'éthylène-alkyle, de ladite composition (A), comprend:
de 25 à 70 % en poids d'éthylène;
de 25 à 50 % en poids d'au moins un acrylate d'alkyle; et
de 5 à 25 % en poids de monoxyde de carbone.

5. Câble selon l'une quelconque des revendications précédentes, dans lequel un alkyle dudit au moins un copolymère sélectionné dans le groupe se composant de monoxydes de carbone d'acrylates d'éthylène-alkyle, de ladite composition (A), est du butyle.

6. Câble selon l'une quelconque des revendications précédentes, dans lequel ledit polyéthylène est un polyéthylène à faible densité.

7. Câble selon l'une quelconque des revendications précédentes, dans lequel l'écran semi-conducteur extérieur (18) comprend en outre:
de 5 à 30 % en poids de NBR; et
de 30 à 40 % en poids de noir de carbone.

8. Mélange de polymères pour préparer un écran semi-conducteur extérieur pour un câble, comprenant :
de 5 à 30 % en poids de NBR ;
de 30 à 40 % en poids de noir de carbone ; et
de 30 à 70 % en poids d'une composition (A) d'au moins un copolymère sélectionné dans le groupe se composant de monoxydes de carbone d'acrylates d'éthylène-alkyle.

9. Mélange de polymères selon la revendication 8, dans lequel ledit au moins un copolymère sélectionné dans le groupe se composant de monoxydes de carbone d'acrylates d'éthylène-alkyle, de ladite composition (A), comprend :
de 25 à 70 % en poids d'éthylène ;
de 25 à 50 % en poids d'au moins un acrylate d'alkyle; et
de 5 à 25 % en poids d'oxyde de carbone.

10. Mélange de polymères selon l'une quelconque des revendications 8 et 9, dans lequel un alkyle dudit au moins un copolymère sélectionné dans le groupe se composant de monoxydes de carbone d'acrylates d'éthylène-alkyle, de ladite composition (A), est du butyle.
